

## UNITED STATES PATENT OFFICE

JOHN J. EGAN, OF BROOKLYN, NEW YORK, ASSIGNOR TO ELECTRIC METALLURGICAL COMPANY, A CORPORATION OF WEST VIRGINIA

## PROCESS OF CASE HARDENING

No Drawing.

Application filed May 26, 1930. Serial No. 455,956.

My invention relates to the production of nitrided layers on metals by heating the metals in nitrogen-containing agents, such as ammonia. It has particular reference to an improved method of forming such hard wear-resistant cases.

The object of my invention is to provide means for accelerating and intensifying the action of nitriding gases on metal articles so as to reduce the time required to produce a case of given hardness or thickness.

The case hardening of alloys is useful as a means of forming hard wearing surfaces on articles to be used for various machine and tool parts. In order to avoid the formation of brittle cases or cause any other deleterious effect upon the material being treated the nitriding process is preferably carried out at low temperatures. To permit the production of a satisfactory case at temperatures of the order of 460° C. to 580° C. it is often customary to alloy with the material to be treated small amounts of a promoting agent such as aluminum or vanadium. A heating period of from 12 to 20 hours in a nitriding atmosphere such as ammonia is usually required to form a suitable case, the length of time of treatment increasing with a decrease in temperature. Such prolonged heating which has been necessary to insure a proper reaction is expensive.

I have found that hard, nitrogen-containing cases may be produced in much less time by the employment of influences acting to ionize the nitriding agent. Such ionizing influence may be generated by an arc, spark, corona or other form of electrical discharge in the nitriding gas in a manner generally similar to the way in which ionizing influences have heretofore been used in chemical synthesis.

In accordance with my invention the specimen to be treated is placed in a suitable chamber containing an atmosphere of ammonia or other nitriding gas, and an electrical discharge is caused to take place within the chamber, preferably in close proximity to the surface of the specimen. The usual nitriding temperature is maintained and the discharge is continued throughout the entire time of

heating. Suitable electrodes across which an arc may be drawn can be easily inserted into the nitriding chamber. A spark such as may be obtained from the ordinary spark plug is an especially convenient form of electrical discharge for this purpose. With one or more spark plugs discharging within the nitriding atmosphere I have been able to produce a case in four hours which is equal in hardness and depth to one produced by the usual nitriding process on a similar metal article in twenty hours.

The speed of the nitriding reaction appears to increase the closer the location of the discharge to the surface of the specimen being treated. I therefore prefer a method in which the specimen itself acts as an electrode and a small arc or spark is drawn from the surface of the metal to one or more other electrodes inserted into the nitriding chamber. By this latter method only two hours treatment is required to produce a hardened layer the equivalent of one formed in thirty or more hours under the same conditions without any ionizing influence.

While I cannot explain precisely the mechanism of the reaction, it appears that the ionizing influence converts the nitriding gas, such as ammonia, into a more active form which accelerates the nitriding reaction. By drawing an arc from the specimen itself the dissociation takes place very near to or directly on the surface of the metal at a point where the active gas may more readily enter into the nitriding reaction before it has time to recombine. This may account in part for the great acceleration obtained by the latter method.

Since other factors may also contribute to produce the results herein shown, the invention should not be restricted by an attempt to describe the theory involved. While the preferred form of ionizing influence consists of an electrical discharge within the nitriding chamber, it will be evident that other means of causing ionization may also be used without departing from the spirit of my invention as defined in the appended claims.

I claim:

1. The method of nitriding metal articles

which comprises heating the articles in the presence of a nitriding agent and subjecting said nitriding agent to an ionizing electrical discharge.

6 2. The method of nitriding metal articles which comprises heating the articles in a chamber containing a nitriding atmosphere and introducing within said chamber an electrical discharge for ionizing said nitriding atmosphere.

10 3. The method of nitriding metal articles which comprises heating the articles in a chamber containing an atmosphere of ammonia and causing an electrical discharge to take place within said chamber.

15 4. The method of nitriding metal articles which comprises heating the articles in a chamber containing an atmosphere of ammonia and causing a spark discharge to take place within said chamber in close proximity to the surface of said articles.

20 5. The method of nitriding metal articles which comprises heating the articles in a chamber containing an atmosphere of ammonia, inserting electrodes within said chamber, and causing a spark discharge between said electrodes while the articles are being heated, said spark being in close proximity to the surface of said articles.

25 30 6. The method of nitriding metal articles which comprises heating the articles in a chamber containing an atmosphere of ammonia, inserting electrodes within said chamber, and drawing a spark between said electrodes and the surface of said articles while they are being heated.

In testimony whereof, I affix my signature.  
JOHN J. EGAN.

which comprises heating the articles in the presence of a nitriding agent and subjecting said nitriding agent to an ionizing electrical discharge.

5 2. The method of nitriding metal articles which comprises heating the articles in a chamber containing a nitriding atmosphere and introducing within said chamber an electrical discharge for ionizing said nitriding atmosphere.

10 3. The method of nitriding metal articles which comprises heating the articles in a chamber containing an atmosphere of ammonia and causing an electrical discharge to 15 take place within said chamber.

4. The method of nitriding metal articles which comprises heating the articles in a chamber containing an atmosphere of ammonia and causing a spark discharge to take 20 place within said chamber in close proximity to the surface of said articles.

5. The method of nitriding metal articles which comprises heating the articles in a chamber containing an atmosphere of ammonia, inserting electrodes within said chamber, and causing a spark discharge between 25 said electrodes while the articles are being heated, said spark being in close proximity to the surface of said articles.

30 6. The method of nitriding metal articles which comprises heating the articles in a chamber containing an atmosphere of ammonia, inserting electrodes within said chamber, and drawing a spark between said 35 electrodes and the surface of said articles while they are being heated.

In testimony whereof, I affix my signature.  
JOHN J. EGAN.

40

#### CERTIFICATE OF CORRECTION.

Patent No. 1,837,256.

Granted December 22, 1931, to

JOHN J. EGAN.

It is hereby certified that the name of the assignee in the above numbered patent was erroneously described and specified as "Electric Metallurgical Company", whereas said name should have been described and specified as Electro Metallurgical Company, as shown by the records of assignments in this office; and that the said Letters Patent should be read with this correction therein that the same may conform to the record of the case in the Patent Office.

Signed and sealed this 9th day of February, A. D. 1932.

(Seal)

M. J. Moore,  
Acting Commissioner of Patents.

**CERTIFICATE OF CORRECTION.**

**Patent No. 1,837,256.**

**Granted December 22, 1931, to**

**JOHN J. EGAN.**

**It is hereby certified that the name of the assignee in the above numbered patent was erroneously described and specified as "Electric Metallurgical Company", whereas said name should have been described and specified as Electro Metallurgical Company, as shown by the records of assignments in this office; and that the said Letters Patent should be read with this correction therein that the same may conform to the record of the case in the Patent Office.**

**Signed and sealed this 9th day of February, A. D. 1932.**

**(Seal)**

**M. J. Moore,  
Acting Commissioner of Patents.**